



wherein R' represents the same radical as R' in the foregoing.

General Formula e



wherein R' represents a member selected from the group consisting of alkyl radicals ( $C_nH_{2n+1}$ ) having 12 to 16 carbon atoms, and  $\text{Me}_2$  represents a member selected from the group consisting of Na and K.

General Formula f



wherein  $n$  is the numerical value of  $4 \leq n \leq 16$ .

General Formula g



wherein  $n$  is the numerical value of  $11 \leq n \leq 15$ .

General Formula h



(phthalic acid and alkyl phthalate)

wherein X represents a radical selected from the group consisting of H and alkyl radicals ( $C_nH_{2n+1}$ ) having 1 to 4 carbon atoms.

General Formula i



(ammonia and amines)

wherein  $\text{R}_1$ ,  $\text{R}_{\text{II}}$  and  $\text{R}_{\text{III}}$  each represents one radical selected from the group consisting of H and alkyl radicals ( $C_nH_{2n+1}$ ) having 2 to 17 carbon atoms.

General Formula j



(aldehyde)

wherein A represents a radical selected from the group consisting of



[of which X and Y each expresses one radical selected from the group consisting of —H, —OH, —NO<sub>2</sub>, —N(CH<sub>3</sub>)<sub>2</sub>, —OCH<sub>3</sub> and —CHCH<sub>2</sub>] and —C<sub>4</sub>H<sub>9</sub>.

These substances, when dissolved and retained in a liquid developer for electrophotography, have the effect of providing said developer with a superb efficiency preventing the occurrence of stained texture on the occasion of developing the copying material.

The exact mechanism involved in preventing or controlling the occurrence of stained texture at the time of development as displayed by said substances represented by metal-dialkyl-dithiophosphates according to the present invention, is not known. However, according to the observation by the inventors of the present invention, said action in case of the negative-to-positive type development can be explained as follows.

By way of example, an electrophotographic copying

material having an electrostatic latent image formed thereon is dipped in a liquid developer wherein metal-dialkyl-dithiophosphate has been dissolved. Thereupon, molecules of said metal-dialkyl-dithiophosphate are influenced by the electric field and cause polarization as follows:



And, in case the residual electric charge of, for example, the non-image area of a copying material is negative, said molecules are repelled electrostatically and migrate to the relatively low-potential portion or the non-potential portion to be adsorbed thereon, and the absorption continues until said portions come to have a potential equivalent to that of their surroundings. Further, as it is conceivable that the molecules of salt are greatly polarized at a portion having high density of electric charge of the copying material, they may be preferentially adsorbed onto the minute portions having low potential in the vicinity of said portion with high density of electric charge. Accordingly, inasmuch as the relatively large image-area whereon the toner is supposed to be adsorbed has an electric charge of quite low density, polarization of said metal-dialkyl-dithiophosphate at this portion can hardly take place, and as a result the adsorption of molecules thereof comes to be nil or quite slight, so that there is no fear of encountering an obstacle in forming images by virtue of said toner. Further, as it is imaginable that the same phenomenon as above may present itself in case of those substances other than said metal-dialkyl-dithiophosphate, too, they are considered as contributable to preventing the stained texture from taking place.

As for the divalent metals to be combined into said metal-dialkyl-dithiophosphate expressed by the foregoing general Formula a and employed for a developer in the present invention, zinc, barium, calcium, strontium, magnesium and the like are suitable. And, as for the preparation of the metal-dialkyl-dithiophosphate as expressed by said general Formula a, there have heretofore been proposed a variety of modes thereof, and said salt is capable of being easily synthesized on the basis of descriptions pertaining to the examples of embodiment appearing in the specifications of, for instance—

German Patent No. 1,018,428  
U.S. Patent No. 2,838,555  
U.S. Patent No. 2,850,452  
U.S. Patent No. 2,895,973  
British Patent No. 822,655  
U.S. Patent No. 2,934,614  
British Patent No. 2,850,453

and, therefore, any further elucidation in this respect is unnecessary.

In addition to the above enumerated salts, there are a variety of compounds with various trade names as follows which comprise some of these salts as principal component, respectively, and have been used commercially as additives for engine oil, and any of them is also suitable for the present invention.

| Trade name    | Name of manufacturer  |
|---------------|-----------------------|
| Santolube 393 | Monsanto Chemical Co. |
| Amoco 193     | Amoco Chemical Co.    |
| OLOA 267      | Olonite Chemical Co.  |

Concrete examples of those substances to be expressed by the aforesaid general Formulas b through j are as enumerated in examples appearing hereunder, and any 70 of the following substances is suitable for the present invention: to wit, any one of phosphates such as disodium-monolauryl-phosphate (general Formula b), sodium-dilauryl-phosphate (general Formula c) and triethyl-phosphate (general Formula d), sulfate such as sodium-lauryl-sulfate (general Formula e), alcohols (general

Formula f) such as nonyl alcohol, isopropyl alcohol,  $\beta$ , Naphthal and cetyl alcohol, monocarboxylic acids (general Formula g) such as lauric acid, myristic acid and palmitic acid, phthalate (general Formula h) such as butylphthalate, amines (general Formula i) such as triethylamine and stearyl amine, aldehyde (general Formula j) such as n-butylaldehyde, cinnamic aldehyde, salicylaldehyde, dihydroxybenzaldehyde, dinitrobenzaldehyde, dimethylaminobenzaldehyde, dimethoxybenzaldehyde and tolualdehyde.

And, the developer of the present invention is obtained by means of kneading at least one of the foregoing substances with pigment, one or more than two resins contributable to imparting polar-controllability, dispersibility and fixability, and a small quantity of organic solvent, and subsequently dispersing the thus kneaded mixture in a carrier liquid (viz. paraffinic hydrocarbon or isoparaffinic hydrocarbon having a electric resistance of more than  $10^{10}\Omega\cdot\text{cm}$ . and a dielectric constant of less than 3). The alternative to said means is to add at least one of the aforesaid substances to either a concentrated liquid developer (prior to dispersion in a carrier liquid) put on the market or a liquid developer for immediate use as available also in the market and mix them well. The suitable quantity of said substance to be employed or the content in the developer in this occasion is in the range of 0.001-0.1 part by weight per 1 part by weight of pigment of a toner contained in the developer. In this connection, it is noted that the quantity of phosphates as expressed by general Formulas b, c and d and the quantity of sulfate as expressed by general Formula e for adding to the developer are sufficient in said range for the sake of effecting a satisfactory result, but as for other substances than the foregoing, the optimum quantity to be added is in the range of 0.01-0.1 part by weight for dithiophosphates as expressed by general Formula a, 0.01-0.05 part by weight for phthalate, 0.001-0.005 part by weight for alcohols, 0.01-0.1 part by weight for carboxylic acid, 0.001-0.005 part by weight for amine, 0.001-0.01 part by weight for Dekalin, 0.01-0.05 part by weight for azobenzene, 0.05-0.1 part by weight for camphor, 0.005-0.05 part by weight for citral, 0.001-0.05 for styrene monomer and 0.001-0.01 part by weight for aldehydes, respectively.

When an electrophotographic copying material is developed with the aforesaid liquid developer according to the present invention, the so-called stained texture incident to development can be almost completely eliminated and, as a result, formation of a fully clear image can be expected. Further, the developer of the present invention has such an advantage that, despite the concentration of image brought about thereby is quite evenly matched with that developed with conventional developers, the resultant image is visually more highly concentrated than the one in the prior art because of the absence of stained texture.

The following is a further elucidation of the present invention with reference to embodiments thereof.

#### DESCRIPTION OF THE PREFERRED EMBODIMENTS

##### Example 1

A mixture having a composition consisting of—

Carbon black -----  
Polar-controlling resin (a manufacture of Japan Gas Chemical Co., Inc., trade name: Nikanol HP-100, principal component: phenol modified xylene resin) -----  
Toluene -----  
5%-toluene solution of metal-dialkyl-dithiophosphate (as expressed by general Formula a wherein  $R_I$ ,  $R_{II}$ ,  $R_{III}$ , and  $R_{IV}$  are isopropyl radicals respectively and Me is zinc) -----

was thoroughly mixed for 16 hours by means of a ball mill, and subsequently 5 g. of thus treated mixture was dispersed in 1,000 cc. of a carrier liquid (a liquid hydrocarbon manufactured by ESSO Standard Sekiyu Co. and having the trade name "Naphtha No. 6"), whereby was obtained a liquid developer for use in electrophotography, said developer containing pigment particles negatively charged. Further, for the sake of comparison of efficiency, another liquid developer for use in said comparison was prepared by similarly dispersing 5 g. of a mixture having the same composition as above but with no metal-dialkyl-dithiophosphate.

Meanwhile, an electrostatic latent image was imparted onto commercially available electrophotographic copying materials through the steps of impressing thereon a negative electric charge according to conventional electrophotography and then laying the negative image upon thus impressed copying materials for subsequent exposure by virtue of a tungsten-filament lamp. After that, the copying materials thus charged with an electrostatic image respectively were employed for forming a copied image by dipping in the liquid developer according to the present invention on the one hand, and by dipping in the developer prepared for the comparison's sake on the other hand, for 25 seconds each. The measurement of the resultant concentration of image area and that of non-image area (viz. the area of stained texture) has led to the following Table 1.

TABLE 1

| Developer                                     | Concentration of— |                |
|-----------------------------------------------|-------------------|----------------|
|                                               | Image area        | Non-image area |
| Developer under the present invention-----    | 1.36              | 0.13           |
| Developer prepared for comparison's sake----- | 1.20              | 0.23           |

In this connection, it is noted that each value of the concentration in the foregoing Table 1 was measured through the relative measurement method, wherein the printing was conducted by employing a 2 mm.-square discontinuous gray scale as the original to avoid the edge effect peculiar to electrophotography and the maximum concentration of the print was measured by comparing it with one having a known concentration.

##### Example 2

A mixture having a composition consisting of—  
G. Carbon black ----- 5  
Polar-controlling resin: Nikanol HP-100 ----- 30  
Resin contributing to dispersibility: Plexol #966 (an  
55 acrylic copolymer resin manufactured by Rohm  
& Haas Co.) ----- 10  
Toluene ----- 45  
5%-toluene solution of metal-dialkyl-dithiophosphate  
(as expressed by general formula wherein both  $R_I$   
60 and  $R_{II}$  are isopropyl radicals, both  $R_{III}$  and  $R_{IV}$  are  
isobutyl radicals, and Me is barium) ----- 10

was thoroughly mixed for 16 hours by means of a ball mill, and subsequently 5 g. of thus treated mixture was dispersed in 1,000 cc. of a carrier liquid (manufactured by ESSO Standard Sekiyu Co. and having the trade name "ISOPAR-H"), whereby was obtained a liquid developer for electrophotography, said developer containing pigment particles negatively charged.

Thus prepared developer was employed for developing electrophotographic copying materials imparted with electrostatic latent images similar to that in case of Example 1 by dipping therein said copying materials, and the resultant prints displayed practically no stained texture.

## Example 3

A mixture having a composition consisting of—

|                                                                                                                                                                                                                  |    |    |
|------------------------------------------------------------------------------------------------------------------------------------------------------------------------------------------------------------------|----|----|
| Carbon black                                                                                                                                                                                                     | 5  | G. |
| Polar-controlling resin: Nikanol HP-100                                                                                                                                                                          | 30 | 5  |
| Resin contributing to dispersibility: Plexol #917 (an acrylic copolymer resin manufactured by Rohm & Haas Co.)                                                                                                   | 10 |    |
| Toluene                                                                                                                                                                                                          | 45 |    |
| 5%-toluene solution of metal-dialkyl-dithiophosphate (as expressed by general formula wherein both $R_I$ and $R_{II}$ are isobutyl radicals, both $R_{III}$ and $R_{IV}$ are lauryl radicals, and Me is calcium) | 10 |    |

was treated in the same way as Example 1, whereby was obtained a liquid developer for electrophotography.

G. 10

15

developers. On the other hand, for the purpose of comparing the efficiency of developers, a developer for use in comparison was prepared by means of dispersing about 5 g. of the mixture having the aforesaid composition in a carrier liquid. Each of the above developers was then treated in the same way as Example 1 and employed for developing the electrophotographic copying material carrying the electrostatic latent image, and subsequently measurement was conducted of the concentration of the resultant images as well as the concentration in the texture area.

The above-stated compositions of developers and the results of measurement with respect to the efficiency of those developers are as put together, in the following Table 2. In this context, it is noted that, notwithstanding there was employed—for respective developer according

TABLE 2

| Developer number | Name of Additive                                                                                                   | Quantity added to basic composition (g.) | Concentration of— |
|------------------|--------------------------------------------------------------------------------------------------------------------|------------------------------------------|-------------------|
|                  |                                                                                                                    |                                          | Image area        |
|                  |                                                                                                                    |                                          | Texture area      |
| 1                | Triethyl phosphate (6% toluene solution)                                                                           | 5                                        | 0.20              |
| 2                | Monolauryl phosphate (5% toluene solution; a manufacture of Nikko Chemicals, Inc., with the trade name Nikkol-SLP) | 5                                        | 0.11              |
| 3                | Dilauryl phosphate (1% toluene solution)                                                                           | 1                                        | 0.09              |
| 4                | Dilauryl phosphate (5% toluene solution; a manufacture of Nikko Chemicals, Inc., with the trade name Nikkol-DLP-4) | 5                                        | 0.13              |
| 5                | Dilauryl phosphate (6% toluene solution)                                                                           | 1                                        | 0.09              |
| 6                | do                                                                                                                 | 10                                       | 0.11              |
| 7                | Na-lauryl phosphate (5% toluene solution; a manufacture of Nikko Chemicals, Inc., with the trade name Nikkol-SLS)  | 5                                        | 0.11              |
| 8                | K-lauryl sulfate (5% toluene solution; a manufacture of Nikko Chemicals, Inc., with the trade name Nikkol-KLS)     | 5                                        | 0.11              |
| 9                | Na-cetyl sulfate (5% toluene solution; a manufacture of Nikko Chemicals, Inc., with the trade name Nikkol-SCS)     | 5                                        | 0.09              |
| 10               | Na-lauryl sulfate (1% toluene solution)                                                                            | 1                                        | 0.11              |
| 11               | Na-lauryl sulfate (5% toluene solution)                                                                            | 1                                        | 0.11              |
| 12               | do                                                                                                                 | 10                                       | 0.11              |
| 13               | Monomethyl phthalate (5% toluene solution)                                                                         | 1                                        | 0.15              |
| 14               | Dibutyl phthalate (5% toluene solution)                                                                            | 5                                        | 0.11              |
| 15               | do                                                                                                                 | 1                                        | 0.11              |
| 16               | Phthalic acid (5% toluene solution)                                                                                | 1                                        | 0.13              |
| 17               | Isopropyl alcohol (0.1% toluene solution)                                                                          | 5                                        | 0.09              |
| 18               | do                                                                                                                 | 1                                        | 0.09              |
| 19               | Cetyl alcohol (0.1% toluene solution)                                                                              | 5                                        | 0.11              |
| 20               | Nonyl alcohol (0.1% toluene solution)                                                                              | 5                                        | 0.13              |
| 21               | Lauric acid (5% toluene solution)                                                                                  | 5                                        | 0.11              |
| 22               | Myristic acid (5% toluene solution)                                                                                | 5                                        | 0.09              |
| 23               | Palmitic acid (5% toluene solution)                                                                                | 5                                        | 0.11              |
| 24               | do                                                                                                                 | 1                                        | 0.13              |
| 25               | do                                                                                                                 | 10                                       | 0.11              |
| 26               | Triethyl amine (0.1% toluene solution)                                                                             | 5                                        | 0.11              |
| 27               | Stearyl amine (0.6% toluene solution)                                                                              | 1                                        | 0.11              |
| 28               | do                                                                                                                 | 5                                        | 0.11              |
| 29               | Dekalin (5% carbon tetrachloride solution)                                                                         | 5                                        | 0.11              |
| 30               | Dekalin (1% carbon tetrachloride solution)                                                                         | 5                                        | 0.11              |
| 31               | Dekalin (0.1% carbon tetrachloride solution)                                                                       | 5                                        | 0.09              |
| 32               | Azobenzene (5% toluene solution)                                                                                   | 5                                        | 0.09              |
| 33               | Azobenzene (1% toluene solution)                                                                                   | 5                                        | 0.11              |
| 34               | Camphor (5% carbon tetrachloride solution)                                                                         | 5                                        | 0.11              |
| 35               | do                                                                                                                 | 10                                       | 0.09              |
| 36               | Citral (6% toluene solution)                                                                                       | 5                                        | 0.11              |
| 37               | do                                                                                                                 | 1                                        | 0.09              |
| 38               | Citral (1% toluene solution)                                                                                       | 1                                        | 0.11              |
| 39               | Styrene monomer (5% toluene solution)                                                                              | 1                                        | 0.09              |
| 40               | do                                                                                                                 | 5                                        | 0.13              |
| 41               | do                                                                                                                 | 0.1                                      | 0.11              |
| 42               | Butyl aldehyde (0.1% toluene solution)                                                                             | 0.1                                      | 0.09              |
| 43               | Cinnamic aldehyde (5% toluene solution)                                                                            | 0.1                                      | 0.09              |
| (1)              |                                                                                                                    | 1.20                                     | 0.23              |

<sup>1</sup> Developer for comparison.

Thus prepared developer displayed a developing effect equivalent to those developers according to the present invention as employed in the foregoing examples.

## Example 4

A mixture having a basic composition consisting of—

|                                                                                                                 |    |    |
|-----------------------------------------------------------------------------------------------------------------|----|----|
| Carbon black (a manufacture of Mitsubishi Kasei Co., Ltd., having the trade name "Mitsubishi #100")             | 5  | G. |
| Polar-controlling resin (a manufacture of Japan Gas-Chemical Co., Inc., having the trade name "Nikanol HP-100") | 40 | 70 |
| Toluene                                                                                                         | 45 |    |

was combined with various additives respectively, and subsequently about 5 g. each of the respective mixtures thus prepared was dispersed in the same carrier liquid as Example 1, whereby were prepared 43 kinds of liquid

to said Table 2—just one additive substance effective in preventing the stained texture, it is definite that, in so far as the quantity employed is in the range of 0.001–0.1 part by weight per 1 part by weight of the pigment contained in a developer, the effect to be brought about in case two substances or more are employed is equivalent to that in case just one substance is employed.

What we claim is:

1. A liquid developer for electrophotography comprising (1) a carrier liquid consisting of a liquid hydrocarbon having an electric resistance of more than  $10^{10}\Omega$  cm. and a dielectric constant of less than 3; (2) a toner dispersed in said carrier liquid, said toner being comprised of carbon black particles and a coating layer coated on said particles, said coating layer consisting essentially of a resin selected from the group consisting of phenol modified xylene resin and acrylic resins; and (3) a stain texture-

preventing agent dissolved in said carrier liquid, said agent being selected from the group consisting of compounds expressed by



in a quantity in the range of 0.01 to 0.1 part by weight per one part by weight of said carbon black, and wherein each of  $\text{R}_1$ ,  $\text{R}_{\text{II}}$ ,  $\text{R}_{\text{III}}$  and  $\text{R}_{\text{IV}}$  is a monovalent radical selected from the group consisting of alkyl radicals having 3 to 18 carbon atoms and aralkyl radicals combined with a side-chain having 3 to 18 carbon atoms, and  $\text{Me}_1$  is a divalent metal radical; compounds expressed by



in a quantity in the range of 0.001 to 0.1 part by weight per one part by weight of said carbon black, and wherein  $\text{R}'$  is selected from the group consisting of H and alkyl radicals having 2 to 12 carbon atoms; compounds expressed by



in a quantity in the range of 0.001 to 0.1 part by weight per one part by weight of said carbon black, and wherein  $\text{R}'$  is the same as  $\text{R}'$  in the preceding Formula b; compounds expressed by



5 in a quantity in the range of 0.001 to 0.1 part by weight per one part by weight of said carbon black, and wherein  $\text{R}''$  is an alkyl radical having 12 to 16 carbon atoms, and  $\text{Me}_2$  is a member selected from the group consisting of Na and K.

10 2. A liquid developer according to claim 1, wherein said agent is a compound of the Formula a and its content in said carrier liquid is in the range of 0.01-0.1 part by weight per part by weight of said carbon black.

15 3. A liquid developer according to claim 2, wherein the metal of the compound expressed in the general Formula a is a member selected from the group consisting of zinc, barium, calcium, strontium and magnesium.

## References Cited

## UNITED STATES PATENTS

|           |        |                       |          |
|-----------|--------|-----------------------|----------|
| 3,241,957 | 3/1966 | Fauser et al. -----   | 252-62.1 |
| 3,079,272 | 1/1963 | Greig -----           | 252-62.1 |
| 3,512,965 | 5/1970 | Matkan -----          | 252-62.1 |
| 3,444,083 | 5/1969 | Oliphant -----        | 252-62.1 |
| 3,076,722 | 2/1963 | Greig -----           | 252-62.1 |
| 3,078,231 | 2/1963 | Metcalfe et al. ----- | 252-62.1 |
| 3,507,679 | 4/1970 | Metcalfe et al. ----- | 252-62.1 |
| 3,528,097 | 9/1970 | Otsuka et al. -----   | 252-62.1 |

20 GEORGE F. LESMES, Primary Examiner

J. P. BRAMMER, Assistant Examiner

U.S. Cl. X.R.

30 35 117-37 LY